

## UNITED STATES PATENT OFFICE

WINSTON F. STOODY, OF WHITTIER, AND THOR RELLING, OF BELVEDERE GARDENS, CALIFORNIA, ASSIGNORS TO STOODY COMPANY, OF WHITTIER, CALIFORNIA, A CORPORATION OF CALIFORNIA

## METHOD OF MAKING METAL CARBIDES

No Drawing.

Application filed May 28, 1930. Serial No. 456,806.

This invention relates to a method of making carbides of metals, and more particularly to a method of making a tungsten carbide of any predetermined carbon content.

5 Tungsten carbide has long been known as an extremely hard, brittle composition, its hardness approaching and being comparable with that of the diamond.

The compound has been shaped, or has 10 been combined with other metals and alloys, the metals and alloys acting as binders, for use as cutting tools for high speed practice. It has also been utilized alone or in combination with other metals and alloys as hard 15 surfacing and insert materials to withstand extreme abrasive wear on oil well drilling bits and the like.

Tungsten carbide made by the fusion process in an electric furnace, has been known 20 since Moisson, Williams and other contemporaries; and later, Lohmann and others successfully made a tungsten carbide by a sintering process, i. e., the temperature range being well below the melting point of 25 tungsten and carbon.

Attention has not been directed in the art to any particular carbide beyond the fact 30 that a carbide was formed, the usual procedure being to add to the powdered tungsten an abundance of carbon with a consequent forming of a tungsten carbide of formula WC with a theoretical carbon content of 6.12 per cent. Moisson, in his experiments on 35 tungsten carbide in the electric furnace, fixes a carbide of the formula  $W_2C$  with theoretical carbon content of 3.16, which later was affirmed by Ruff and Wunsch in 1914, who also noted various eutectics which apparently occurred starting with a carbon content of 40 0.43 per cent.

Through quite extended research and experimentation on the formation of tungsten carbides, we have devised a method of forming the carbides of any desired carbon content 45 without the use of any appreciable over-

abundance of carbon, and have evolved carbides of various carbon content answering to the theoretical known carbides and eutectic points noted by former experimenters. The theory of the composition occurring at 50 eutectic points containing less than 6.12 per cent combined or dissolved carbon, is not understood; but we believe the composition at these points is a conglomerate of tungsten carbide of the formula  $W_2C$ , and tungsten 55 with a case hardened shell of tungsten carbide of formula  $W_2C$ , because after the tungsten carbide is separated from the original composition, the remainder upon grinding, dissociates into tungsten and  $W_2C$ , thereby denoting that all of the tungsten has not 60 been completely changed into a carbide, but that some has been merely coated with a covering or shell of carbide. These carbides or eutectic points were obtained by varying the 65 percentage of carbon in the mixture and sintering in a gas furnace at temperatures ranging from 1700° F.-2250° F. Eutectic points occurring at points above the combined or dissolved carbon content of 6.12 per cent, 70 were noted at temperatures ranging from 2500° F. upwards in a glo-bar electric furnace.

The essence of our invention then consists 75 in a method of intimately mixing the tungsten powder and carbon so that all the tungsten is in intimate contact with the required amount of carbon to produce the required tungsten carbide of specific carbon content, and also means for controlling the 80 variables, viz., the percentage of carbon brought into intimate contact with the metallic powder to be carbonized; the duration or time of heat treatment; and the temperature at which the heat treatment is 85 made.

Our invention consists in the steps of the method hereinafter described and claimed.

To gas carbon black, we add sufficient petroleum oil to give the required consistency to 90

make a working paste. The mixture is given a long and thorough mixing in a paste-mixing machine used for intimately mixing powders, and has been found satisfactory. Other ag-  
5 glutinants such as sugar solutions, starch, resin and the like, have been used before, but they all have a tendency to increase the carbon content of the mixture not readily susceptible of control. It is an essential ele-  
10 ment of our method, that we use a distilled petroleum oil so that the carbon added to the tungsten, may be definitely weighed and determined, and no appreciable increase in the carbon content of the tungsten carbide com-  
15 position will result. The petroleum oil being a distilled product, will distill off upon subsequent heating, and leave no additional carbon in the tungsten carbide. Other volatile agglutinants which wholly volatilize dur-  
20 ing the subsequent heating, may be used. To this paste is then added the proper proportion of very fine, pure tungsten powder, the resulting mass being then mixed thoroughly in a mechanical mixing machine for one to  
25 three hours, until every particle of tungsten has a coating of carbon. The product is then packed in refractory molds or crucibles, covered with a layer of graphite to prevent oxidation, and given a sintering heat treatment in either an electric or gas furnace of sufficient heat degree and length of time to insure the formation of the carbide.

A typical charge which gives a tungsten carbide of theoretical carbon content of 6.12, would be as follows:

93.8 pounds tungsten powder.  
6.2 pounds carbon contained in paste.

40 For any other lower carbides or eutectic points, the percentage would be varied so as to approach the theoretical carbon content of the lower carbides or eutectic points.

We have described our method relating to  
45 the making of tungsten carbides for eutectics of predetermined carbon content. However, the same method may be used in the production of carbides and eutectics of predetermined carbon content of metals other than tungsten. The temperature required for sintering in connection with metals other than tungsten, will, of course, vary with the particular kind of metal used.

Various changes may be made by those skilled in the art, in the steps of the method without departing from the spirit of our invention as claimed.

We claim:

1. A method of making carbides of metals, comprising making a paste of carbon with distilled petroleum oil, intimately mixing the paste with a finely divided metal, and sintering the mixture.

66 2. A method of making a carbide of tung-  
sten, comprising making a paste of carbon

and distilled petroleum oil, intimately mixing the paste with finely divided tungsten, and sintering the mixture.

3. A method of making a carbide of tung-  
70sten with a definite carbon content to corre-  
spond to an eutectic point, comprising mak-  
ing a paste of carbon and distilled petroleum  
oil, intimately mixing a definite proportion  
75 of carbon of said paste with a definite per-  
centage of finely divided tungsten, and sin-  
tering the mixture.

In testimony whereof we have signed our  
names to this specification.

WINSTON F. STOODY.  
THOR RELLING.

70

75

80

85

90

95

100

105

110

115

120

125

130